

# UNITED STATES PATENT OFFICE.

BENJAMIN F. LOVELACE, OF BALTIMORE, MARYLAND.

## METHOD OF PRODUCING OXID OR OXIDS OF MANGANESE.

1,352,208.

Specification of Letters Patent. Patented Sept. 7, 1920.

No Drawing.

Application filed April 24, 1919. Serial No. 292,390.

To all whom it may concern:

Be it known that I, BENJAMIN F. LOVELACE, a citizen of the United States, and residing at Baltimore, Maryland, have invented certain new and useful Improvements in Methods of Producing Oxid or Oxids of Manganese, of which the following is a specification.

This invention relates to the production of oxids of manganese, more especially a mixture of oxids which is capable of easily liberating a portion of its oxygen, and which consists principally of manganese dioxid with varying percentages of the lower oxid or oxids of manganese.

It is the object of this invention to produce an oxid or mixture of oxids which by reason of its physical and chemical characteristics is especially adapted for use in preparing the mixtures of oxids, known as hop calite, having extremely desirable catalytic properties; which catalysts are described in the application of Frazer *et al.* Serial No. 275,007, filed Feb. 4, 1919. The oxids of manganese prepared by my process are in an extremely, finely divided state, are substantially completely hydrated, show a high degree of catalytic activity, and can be very cheaply produced.

In carrying out the present invention, I provide a process wherein manganese is electrolytically oxidized to form the desired oxids of manganese. More specifically, I electrolyze a solution of suitable salts in a single compartment cell with an anode containing manganese. In the prior processes wherein a solution such as of alkali hydroxids or carbonates were used as electrolytes with an anode containing manganese, the object has been to produce permanganates. In cells of such a character a diaphragm is used to separate the anolyte from the catholyte in order to prevent the subsequent reduction at the cathode of permanganate formed at the anode. By my process I eliminate the diaphragm, using a single compartment cell and thus the permanganate formed at the anode is allowed to move freely to the cathode where the permanganate is practically quantitatively reduced to the hydrated oxids contemplated by this invention. Some oxids are produced at the anode by the partial oxidation of the manganese of the anode.

Various electrolytes such as various soluble salts as the carbonates and bicarbonates of

the alkali metals or ammonium may be used but I have found that a solution of the ordinary commercial ammonium carbonate, which usually contains some bicarbonate and carbamate, gives the best results. The anode may be ordinary ferromanganese or other manganese containing alloys such as are described and claimed in my patents, numbers, 1,291,680, 1,291,681, 1,291,682, dated Jan. 14, 1919, or other manganese containing alloys, and as cathode I prefer to use iron. I have found that by using a temperature below 35° C., very satisfactory results are obtained. Better results are obtained at lower temperatures such as 12° C., or lower, but the use of such temperatures may be commercially infeasible on account of the cost of refrigeration. I also employ a current density of 0.10 to 0.15 amperes per square centimeter using preferably an anode consisting of ordinary commercial ferromanganese. The conditions under which the electrolysis takes place such as temperature, concentration of electrolyte, composition of the anode, current density, etc., may be varied within wide limits with satisfactory yields of hydrated oxids.

As the electrolysis proceeds, using for example, a saturated or very nearly saturated solution of commercial ammonium carbonate with a manganese containing anode, the manganese goes into solution with the formation of ammonium permanganate at the anode and with some deposition of hydrated oxids of manganese; the permanganate goes to the cathode where it is reduced to form the bulk of the hydrated oxids of manganese. An analysis shows that the oxids formed contain variable amounts of hydrated oxids of iron due to the iron in the anode. The available oxygen in the mixed oxids is somewhat less than that corresponding to manganese dioxid. The product thus obtained is very finely divided and when filtered, washed and mixed with certain other oxids such as those of silver, copper and cobalt gives a material which has very marked catalytic properties.

In place of the ammonium carbonate I may use carbonates or bicarbonates of other alkali metals such as sodium, potassium or lithium with satisfactory results but the best results are obtained when ammonium compounds are used, and I use the term "alkali metal" to include ammonium. I do not intend to limit myself to the specific salt described, but I claim the process of electro-

lyzing a soluble compound with a manganese containing anode, broadly, except as limited by the following claims.

Having thus described my invention, I 5 claim:

1. A process of producing an oxid or oxids of manganese comprising electrolyzing with an anode containing manganese in a single compartment cell a solution of an 10 ammonium salt containing the  $\text{CO}_3$  radical.

2. A process of producing an oxid or oxids of manganese comprising electrolyzing with a manganese containing anode in a single compartment cell a solution of am- 15 monium carbonate.

3. A process of producing an oxid or oxids of manganese comprising electrolyzing with a manganese containing anode at a temperature below 35° C. a solution which 20 shows an alkaline reaction toward litmus.

4. A process of producing an oxid or oxids of manganese comprising electrolyz- 25

ing with a manganese containing anode in a single compartment cell at a temperature below 35° C. a solution which shows an al- 25  
kaline reaction toward litmus.

5. A process of producing an oxid or oxids of manganese comprising electrolyzing with a manganese containing anode at a temperature below 35° C. a solution of a 30 salt having the  $\text{CO}_3$  radical.

6. A process of producing an oxid or oxids of manganese comprising electrolyzing with a manganese containing anode in a single compartment cell at a temperature 35 below 35° C. a solution of a salt having the  $\text{CO}_3$  radical.

7. A process of producing an oxid or oxids of manganese comprising electrolyzing with a manganese containing anode in a 40 single compartment cell at a temperature below 35° C. a solution of ammonium car-  
bonate.

BENJAMIN F. LOVELACE.